

Patented Aug. 18, 1953

2,649,367

# UNITED STATES PATENT OFFICE

2,649,367

## CADMIUM-FREE LOW FUSING POINT ALLOY

Albert A. Smith, Jr., Metuchen, and John L. Everhart, Linden, N. J., assignors to American Smelting and Refining Company, New York, N. Y., a corporation of New Jersey

No Drawing. Application October 7, 1950,  
Serial No. 189,044

1 Claim. (Cl. 75—134)

**1**  
This invention relates to alloys and more particularly to low fusing point alloys.

It is an object of the invention to provide cadmium-free, low melting point alloys.

In accordance with the invention, alloys are provided comprising, by weight, 32-34% Bi, 42-44% In, 7-8% Pb and 15-18% Sn, and have fusing points of approximately 59° C.

It will be observed from the compositions that these alloys do not contain cadmium and, accordingly, they are particularly suitable for certain applications as heat transfer media where cadmium would be detrimental.

What is claimed is:

Low melting point alloys composed of 32-34% Bi, 42-44% In, 7-8% Pb and 15-18% Sn. 15

ALBERT A. SMITH, JR.  
JOHN L. EVERHART.

**2**

References Cited in the file of this patent

## UNITED STATES PATENTS

| Number      | Name | Date          |
|-------------|------|---------------|
| 5 2,218,153 | Pray | Oct. 15, 1940 |

## OTHER REFERENCES

French, Industrial and Engineering Chemistry, vol. 27, December 1935; pages 1464 and 1465.

Smith, Metal Industry, October 26, 1945; page 262.

"Fusible Alloys Containing Tin," September 1949, 24 pages, page 3 relied on. Published by the Tin Research Institute, Columbus, Ohio.